

## UNITED STATES PATENT OFFICE

2,290,024

## ALUMINUM ALLOY

Walter Bonsack, South Euclid, Ohio, assignor to  
The National Smelting Company, Cleveland,  
Ohio, a corporation of Ohio

No Drawing. Application February 20, 1942,  
Serial No. 431,681

8 Claims. (Cl. 75—146)

This application is a continuation-in-part of my copending application Serial No. 389,020, filed April 17, 1941. The invention relates to alloys, and particularly to aluminum base alloys suitable for casting and working and having high strength at ordinary and elevated temperatures.

It is an object of this invention to produce alloys having relatively high elongation and relatively high tensile strength.

It is a further object of this invention to provide a relatively light alloy which may be easily cast and machined, which may be used at elevated temperatures without a rapid deterioration of desirable properties, and which may be readily treated with anodic treatment to give excellent lustre and finish.

It is a still further object of this invention to provide an alloy having a relatively high proportional limit and relatively high fatigue strength, and in which these properties may be obtained without heat treatment.

When magnesium and zinc are added to aluminum in the proper proportions, a ternary compound of aluminum, magnesium and zinc is formed, which compound is soluble in solid solution in the aluminum. The presence of this compound in a relatively small amount greatly improves the characteristics of aluminum and produces an alloy having high strength combined with high ductility, good casting, rolling, extruding and forging properties, good color and excellent corrosion resistance. In calculating the amount of magnesium and zinc that should be present in the aluminum alloy to form the desired percentage of ternary compound, only magnesium which is not combined with silicon is to be calculated, as it is only such magnesium that is available to combine with zinc and aluminum to form the ternary compound.

The ternary compound is said by some investigators to have a composition having substantially the formula  $Al_3Mg_2Zn_5$ , and other investigators have considered the formula for the ternary compound as being  $Al_2Mg_3Zn_3$ . It will be seen that the amounts of magnesium and zinc relative to each other are quite similar in both formulae. The magnesium and zinc should be present in about the proportion necessary to form the ternary compound of either formula or, preferably, the ratio of the magnesium to zinc in the alloy should be between the ratios in the formulae.

An excess of zinc, over and above that which cooperates with magnesium and aluminum to

form a ternary compound according to the above formula having the greatest proportion of zinc, increases the brittleness and decreases the ductility of the alloy. For this reason it is undesirable that zinc be present in quantities substantially greater than the amount to react to form such a ternary compound with magnesium and aluminum. The most desirable properties are obtained when the magnesium and the zinc are proportioned so that the ratio of magnesium (uncombined with any silicon) to zinc is about equal to the ratio represented by the formula  $Al_2Mg_3Zn_3$ , or somewhat larger as represented by the formula  $Al_3Mg_2Zn_5$ . A small amount of magnesium may be provided to replenish losses that may occur when the alloy metal is remelted.

Magnesium adds to the hardness and machining qualities of the alloy and, as above stated, should be present in an amount sufficient to combine with the zinc and aluminum present. In greater quantities, magnesium tends to make the alloy sluggish, decreasing castability.

The improved aluminum alloys may have the ternary compound of aluminum, zinc and magnesium present in an amount ranging from about 2% to 20%, the preferred range being between about 3% and 15%. At room temperature the ternary compound goes into solid solution in aluminum alloys in an amount of about 2%. The percentage in solid solution increases at high temperatures and decreases upon cooling, the excess precipitating out. Aluminum alloys containing the ternary compound may, therefore, be advantageously heat treated to improve their properties.

A small amount of silicon is usually present in aluminum alloys and up to 1.5% silicon may be present in the alloys of the present invention. If the alloys are to be rolled or worked the silicon should be low, from about the minimum obtainable quantity of .04% or .05% to about .7%. More than .7% is frequently desirable in casting alloys. Silicon combines with magnesium in preference to most elements, each part by weight of silicon combining with about 1.75 parts, by weight, of magnesium to form  $Mg_2Si$ . At least sufficient magnesium is therefore added to the alloy to combine with the silicon uncombined with any calcium to form  $Mg_2Si$ , and in addition to combine with all the zinc and form the ternary compound according to the formula  $Al_2Mg_3Zn_3$ .  $Mg_2Si$  is more stable than the ternary compound above mentioned and may be maintained in solid solution in aluminum alloys in an amount up to about 1.85%, which is the quantity of  $Mg_2Si$

present if the silicon is present in the alloy, and acts as a hardener which is sometimes desirable in conjunction with the ternary compound.  $Mg_2Si$  does not, however, make as efficient use of the magnesium as does the above mentioned ternary compound. Therefore, it is desirable to have the magnesium present on the rich side to prevent the silicon from being present in excess and taking magnesium away from the ternary compound.

It has now been found that aluminum alloys containing magnesium (over that necessary to combine with silicon) and zinc in the proportions to form a ternary compound are greatly improved by the addition of about .05% to 1.5% manganese, about .05% to 1.5% chromium and about .1% to 1.5% nickel, with one or more of the grain refining elements, such as those selected from the group consisting of titanium, columbium, zirconium, boron, tungsten, molybdenum, tantalum and vanadium in a total amount of .005% to .5%. Iron may be present in an amount from about .1% to 1.5%.

Although the metals manganese, chromium and nickel each increase the hardness of the alloy, a given percentage of each of these elements improves certain of the properties more than it does others. Nickel increases the tensile strength, proportional limit and yield strength of the alloy without decreasing its elongation to any appreciable degree. In fact, with certain amounts of nickel the elongation is increased, so that an alloy having exceedingly desirable and exceptional properties may be obtained.

Alloys containing nickel may be readily heat treated or age hardened to give somewhat superior properties, but very desirable properties which are almost equivalent to the heat treated alloys are also obtained when castings are simply aged at room temperature, with or without quenching from the mold.

Nickel is quite an effective element in the alloy and appreciable improvements in properties of the alloy are noted when it is present in an amount of about 1%, or more. The preferred properties are obtained with about .3% to about .8% or 1% nickel, and in some cases it is desirable to have the nickel present in amounts as great as 1.5%.

Manganese, although it decreases the tensile strength and elongation to some degree, increases the yield strength, hardness and proportional limit of the alloy. It also makes the alloy more corrosion resistant.

Alloys containing manganese may be readily heat treated or age hardened to give somewhat superior properties, but very desirable properties are obtainable when castings are simply aged at room temperature, or when quenched from the mold and aged.

Manganese is a very effective element in the alloy and desirable improvements are noted when about 1% or even a little less, such as .05%, is present in the alloy. The preferred properties are obtained with about .2% to about .5% or .8% manganese, and in some cases it is desirable to have the manganese present in amounts as great as about 1%, or even 1.5%.

Chromium is a particularly effective alloying element in the alloy of the present invention. Although it does not appear to improve the proportional limit and yield strength of the alloy quite as much as does manganese, it increases the elongation and further increases corrosion resistance. It is, therefore, particularly ad-

vantageous that both chromium and manganese be present. As little as .05% or 1% chromium, and particularly with manganese, is effective in improving the properties of the alloy, but .2% or .3% to about 1%, or even 1.5%, is desirable. When manganese is also present, the total of manganese and chromium should preferably be between about .3% and 2.5% of the alloy.

The quantity of each of the hardening metals desired in a given alloy also depends somewhat upon the quantity of other hardening ingredients present and upon the amount of ternary compound, a given hardness and tensile strength often being obtainable either with a relatively large amount of strength-improving hardening metal and a relatively small amount of ternary compound, or with a relatively small amount of such metal and a relatively large amount of magnesium and zinc in the proportions of a ternary compound.

An alloy containing 2%, or even as little as 1%, of the ternary compound may be used for casting purposes. The castability, however, is improved with an increase in the amount of ternary compound and it is, therefore, preferred to have a larger percentage of the ternary compound present, such as 4% to 8% or 9% for casting purposes, 9% ternary compound containing about 5.4% zinc. When the casting is more or less intricately shaped, still greater percentages, such as 10% to 12% or 15%, of the ternary compound may be present. For alloys to be forged or shaped after casting, the ternary compound should be present in the lower ranges, such as 2% to 8% or so, as the metal is less hard with the lower percentages of the ternary compound.

A larger proportion of the ternary compound may be present in alloys which are to be given a so-called "solution treatment" than in alloys to be given only an aging treatment, or those to be quenched from the casting mold and aged at relatively low temperatures. Thus, the desirable properties of the solution heat treated alloys may be obtained when they contain the ternary compound in amounts up to 15% or so, whereas less of the ternary compound, such as 4% to 6%, is preferred in alloys which are quenched upon removal from the mold and heat treated at a low temperature, or aged at room temperature.

It has generally been considered that aluminum alloys of magnesium containing iron much above the impurity value in commercial aluminum are of little commercial value; but it has also now been found that an alloy containing the magnesium, zinc and silicon proportioned as herein described, and also containing manganese, chromium, nickel and a grain refining metal such as is set forth in the above group, is improved by the presence of iron in suitable proportion.

Iron in suitable amounts further increases the hardness and tensile strength of the alloy without decreasing its ductility a substantial amount. A small amount of iron thus permits one to obtain the properties desired with a smaller amount of magnesium and zinc. Iron also improves castability. These alloys containing iron may be readily heat treated or age hardened to give somewhat superior properties, but the iron in combination with manganese, chromium and the ternary elements in the above proportion is also outstanding in that almost as desirable properties are obtained when castings

are aged at room temperature without a heat treatment or quenching.

Iron has generally been considered to crystallize in large platelike crystals, which weaken the alloy. Iron in the presence of the ternary compound appears to crystallize in finely dispersed form and the ternary compound also seems to be dispersed, thus producing a highly desirable alloy.

The quantity of iron desired in the alloy depends upon the quantity of other hardening ingredients present, upon the amount of ternary present, and upon what properties are most important. A given hardness and tensile strength is often obtainable with a relatively larger amount of iron and a relatively smaller amount of ternary compound, or a relatively smaller amount of iron and a relatively larger amount of ternary. Iron may be present in the alloys of the present invention in amounts between about 0.1% and about 1.5%. With the larger percentage of iron in the alloys, the percentages of manganese and chromium may be reduced considerably. If both manganese and chromium are present in substantial amounts and if workability, ductility and corrosion resistance are not to be impaired, the iron should be low, i. e., about 0.1% or less to about .6% or .7% of the alloy. If yield strength and high tensile strength are most important and ductility less important, the amount of iron may be greater.

The grain refining elements are particularly desirable in an aluminum alloy containing iron, manganese, chromium and the ternary compound. Although the iron itself improves the properties of the alloy, the manganese, chromium and grain refining elements exert a still further improvement independently of iron.

The aluminum alloys of the present invention containing magnesium, uncombined with silicon, and zinc in the proportion of a ternary compound, when cast in molds of a design such that chilling takes place substantially simultaneously in the various portions of the casting, solidify without the use of grain refining agents to form good castings. However, it has been found that certain grain refining elements substantially improve the properties of the aluminum alloy containing the ternary compound, iron, manganese, chromium and nickel. This is especially true when the metal is cast in molds of more or less intricate shape where the chilling may not be so uniform throughout the casting.

The grain refiners which I have found exert greatest improvement in the properties of the alloy are members of the group consisting of boron in the amount of .005% to 1%, zirconium in the amount of .01% to .5%, tungsten in the amount of .01% to .5%, molybdenum in the amount of .01% to .5%, vanadium in the amount of .01% to .5%, titanium in the amount of .05% to .5%, columbium in the amount of .01% to .5% and tantalum in the amount of .05% to .5%. These grain refining elements should preferably be present in a total amount of from .005% to .5% and it is frequently desirable to have more than one of these elements present in a given alloy.

While the grain refiners in the above group are desirable in the alloys of the present invention, not all of the grain refiners affect the properties in the same way. The particular refiner or group of refiners selected in any given instance depends upon the particular condition which must be satisfied. The grain refiners se-

lected from the group consisting of titanium, tungsten, molybdenum, zirconium and vanadium, and especially tungsten and molybdenum, improve both the strength and the elongation of the castings.

Titanium being readily available is frequently used, but when special properties of the fabricated article are important it is desirable to select the grain refiner that is most suitable for such properties. The grain refiners boron, columbium and tantalum may advantageously be used where appearance, finish and corrosion resistance are important.

The above described hardening elements, manganese and chromium, substantially decrease the hot shortness, improve the properties of the alloy and assist in maintaining the improved properties at high temperatures such as are encountered in internal combustion engines. The above grain refining elements, particularly members of the group consisting of zirconium, tungsten, molybdenum, vanadium and titanium, also have this property, particularly when present in larger amounts, such as .2% or .3% or so. It may, therefore, be desirable to have up to .5% or so of these latter elements present.

The following example illustrates the alloys of the present invention.

An aluminum base alloy containing magnesium, zinc and silicon in proportion to form 6% of a ternary compound based on the formula  $Al_2Mg_3Zn_3$ , about .3% manganese, about .25% chromium, about .2% titanium, about .6% iron and about .22% nickel, with the balance substantially all aluminum and minor impurities, was prepared and chill cast into test bars. The test bars, air cooled after removal from the mold and aged seven days at room temperature, had a tensile strength of 40,700 lbs./sq. in., a proportional limit of 18,400 lbs./sq. in., a yield strength of 25,600 lbs./sq. in., a hardness of Rockwell E 81.5 and an elongation of 7.2%.

Copper is frequently an impurity in aluminum alloys and, unlike the hardeners present in alloys of the present invention, copper is a precipitation hardening ingredient which is much more soluble at high temperatures than at low temperatures. Substantial amounts of copper are desirable when the alloy is to be solution heat treated. Alloys of the present type containing copper in an amount of more than .1% or so form the subject matter of copending applications.

Since the molecular proportion of zinc is never more than the molecular proportion of the relatively light magnesium in the ternary compound, it is seen that in addition to high strength the alloys are light in weight and are, therefore, especially adapted to aircraft construction and the like. This is particularly true when the quantity of ternary compound is sufficiently low so that the alloy may be drawn or rolled into structural members.

If the alloy contains uncombined silicon, about 1.75% magnesium is required to combine with each percent of uncombined silicon to form magnesium silicide ( $Mg_2Si$ ) before any ternary compound will be formed. For example, if 2% of the ternary compound on the basis of  $Al_2Mg_3Zn_3$  be desired in an alloy having .3% silicon, the amount of magnesium to be added to form the ternary compound will be .45%, or about .5%, and the magnesium to combine with .3% silicon will be about .5%, making a total of about 1%.

The magnesium and zinc in an alloy containing .7% free silicon and 20%  $Al_2Mg_3Zn_3$  would be

about 7% and 12%, respectively. The alloys described herein include aluminum, magnesium and zinc, the magnesium, uncombined with silicon, being proportioned to the zinc in the ranges of the formulae given for the ternary compound. The proportions for the formation of the ternary compound in the alloy exist when the magnesium is about 35% to 45% of the zinc content plus 175% of the silicon content. Most desirable properties may be obtained when the magnesium (uncombined with silicon) is in the lower portion of this range, or about 35% to 40% of the zinc.

In the above example of alloys of the present invention, it is to be noted that excellent tensile strength and hardness are obtainable in a relatively short time by aging at room temperature. A very astounding fact has been discovered, however, in connection with these alloys, namely, that the tensile strength may increase up to approximately 50% of its initial value by aging at room temperature for relatively long periods of time, such as a few months. The same improvement in tensile strength can, of course, be obtained relatively quickly by aging at temperatures above room temperature.

To obtain properties even of the same order of magnitude in aluminum base alloys commonly in use, one has to resort to a solution and aging heat treatment, whereas in alloys of the present invention it is not necessary to solution heat treat 30 for improvement in properties.

The alloys of the present invention have good fatigue and tensile strength and a relatively high proportional limit, even at relatively high temperatures; they have to be heat treated if it is desired to improved and modify their properties, although such heat treatment is not required; and they have sufficient ductility and hardness so that they can be rolled or formed into sheets, rods, wire, structural shapes, castings, machine parts, etc. These alloys have a desirable color, high corrosion resistance, and may be anodically finished or highly polished with excellent results, and are suitable for many uses, among them being the production of castings which are shaped or formed to some extent after casting. The alloys having the lower percentages of ternary compound may even be forged at room temperature and are thus useful for many special purposes.

As pointed out above, grain refiners are usually desirable in alloys of the present invention. However, it has been found that the alloys of the present invention have relatively high strength, high proportional limit and ductility without solution heat treatment, even in the absence of the grain refiners. The alloys may be cast, rolled, forged or otherwise shaped with or without grain refiners.

It is to be understood that in considering the amount of zinc and magnesium to add to aluminum alloys to form the ternary compound of aluminum, magnesium and zinc in the alloy, such magnesium as is necessary to combine with the uncombined silicon is not to be considered as part of the magnesium necessary to form the specified amount of ternary compound.

It is to be understood that the particular compounds disclosed and the procedure set forth are presented for purposes of explanation and illustration, and that various equivalents can be used, 5 and modifications of said procedure can be made without departing from my invention as defined in the appended claims.

What I claim is:

1. An aluminum base alloy containing magnesium, zinc, about .1% to about 1.5% iron, about 10 .05% to 1.5% manganese, about .05% to about 1.5% chromium, about .1% to 1.5% nickel, silicon in an amount up to 1.5%, and one or more grain refining metals, with the balance substantially all aluminum and minor impurities, the amount of zinc in the alloy being about .6% to about 9%, and the amount of magnesium in the alloy uncombined with silicon being about 35% to about 45% of the zinc content, the total magnesium being within the range of about .5% to about 7%.

2. An aluminum base alloy containing magnesium, zinc, about .1% to about 1.5% iron, about 15 .05% to 1.5% manganese, about .05% to about 1.5% chromium, about .1% to 1.5% nickel, silicon in an amount up to 1.5%, and one or more grain refining metals in a total amount of about .005% to about .5%, with the balance substantially all aluminum and minor impurities, the amount of zinc in the alloy being about .6% to about 9%, and the amount of magnesium in the alloy uncombined with silicon being about 35% to about 45% of the zinc content, the total magnesium being within the range of about .5% to about 7%.

3. The alloy set forth in claim 1 in which the zinc content is about 1.2% to 6% and the magnesium content is within the range of about .5% to 6%.

4. The alloy set forth in claim 1 in which the zinc content is about 1.2% to 4.8%, and the magnesium content is within the range of about .5% to 5%.

5. The alloy set forth in claim 2 in which titanium is present in the amount of about .05% to .5%.

6. The alloy set forth in claim 2 in which molybdenum is present in the amount of about .01% to .5%.

7. The alloy set forth in claim 2 in which zirconium is present in the amount of about .05% to .5%.

8. An aluminum base alloy containing magnesium, zinc, about .1% to about 1.5% iron, about 55 .05% to 1.5% manganese, about .05% to about 1.5% chromium, about .1% to 1.5% nickel, and silicon in an amount up to 1.5%, with the balance substantially all aluminum and minor impurities, the amount of zinc in the alloy being about .6% to about 9%, and the amount of magnesium in the alloy uncombined with silicon being about 35% to about 45% of the zinc content, the total magnesium being within the range of about .5% to about 7%.

WALTER BONSACK.